

R. E. BRADLEY,  
BILLET CASTING,  
APPLICATION FILED MAR. 20, 1920.

1,393,195.

Patented Oct. 11, 1921.

Fig. 1.



Fig. 2.



Fig. 4.



Fig. 3.



Fig. 5.



Inventor  
Ross Edward Bradley,  
By Swanson date  
his Attorney

# UNITED STATES PATENT OFFICE.

ROSS EDWARD BRADLEY, OF ROLAND PARK, MARYLAND.

## BILLET-CASTING.

1,393,195.

Specification of Letters Patent. Patented Oct. 11, 1921.

Application filed March 20, 1920. Serial No. 367,525.

To all whom it may concern:

Be it known that I, Ross EDWARD BRADLEY, a citizen of the United States, residing at Roland Park, in the county of Baltimore, 5 State of Maryland, have invented a new and useful Billet-Casting, of which the following is a specification.

My invention relates to improvements in billet casting. The object is to provide improved method and means for casting a hollow or approximately hollow cylindrical metal billet.

The invention is especially applicable to casting billets of copper, or the alloys there- 15 of, for use in tube drawing.

The invention contemplates the elimination of the sand core and the substitution of a metallic core so devised and arranged as to yield to the pressure of the surrounding 20 billet, due to its contraction in cooling, in order to prevent the cracking or breaking of the billet, as would ordinarily be the case were the billet allowed to cool and contract about a rigid metallic core.

25 Referring to the drawings, which illustrate merely by way of example, suitable means for effecting my invention:—

Figure 1 is a vertical section of a mold and core embodying my invention, in position for casting.

Fig. 2 is an elevation of the core which is preferably of sheet metal.

Fig. 3 is a horizontal section on line 3—3 of Fig. 2.

Fig. 4 is a sectional elevation of a mold provided with another form of collapsible core embodying my invention.

Fig. 5 is a cross-section of the core shown in Fig. 4.

40 Similar numerals refer to similar parts throughout the several views.

As shown in Figs. 1 and 4, the mold 10 is suitably supported on the trunions 11 and is provided at the top with the pouring cup 12, and at the bottom with the block or core bit 13, which serves to close the bottom of the mold and to centralize the lower end of the core 14. Suitable means, such as pin 15, is provided for holding the block 13 in 50 position during the molding operation.

The pouring cup 12 is provided with the apertures 16 arranged around the upper end of the mold for permitting the flow of metal from the cup into the mold.

55 In Figs. 1, 2 and 3, the core 14 consists of a flexible sheet metal cylinder, having its

side edges or margins 17 and 18 adapted to overlap. The lower end of this sheet metal core rests in the counter-sunk portion of block 13, the outer margin of said counter-sunk portion forming means for limiting the expanding movement of the said core. This supporting block in no way interferes with the free contraction of the core, due to the contraction of the metal, as it cools. In 60 like manner the spaced lugs or projections 12', extending radially from the inner wall of the lower flange of funnel member 12, engage the upper periphery of the core, to limit its expanding movement at this end, 65 without interfering with its free contraction.

In operation, with a device as shown in Figs. 1, 2 and 3, the billet is cast by pouring the metal into the cup 12, and through 75 the aperture 16, until the mold has been filled to approximately the level of said apertures.

The cup 12 and the block 13 are then removed and the mold turned on its trun- 80 nions, and after the billet has sufficiently set the same with the core inclosed thereby is forced from the mold.

The billet may then further cool and contract without danger of injury, because of 85 the collapsible or yielding character of the sheet metal cylindrical core 14. This core is afterward forced out of the billet in any suitable way.

In the structure shown in Figs. 4 and 5 90 the mold and pouring cup are substantially the same, while the core is composed of the elements 21, 22 and 23. These elements have the relative cross-section substantially as shown in Fig. 5. The middle element 22 is 95 wedge shaped, and is provided with the feathers or ridges 24, seated in corresponding grooves in the elements 21 and 23, for maintaining the said three elements in required relative cross-sectional position. It 100 will be understood that the elements 21 and 23 are correspondingly tapered to accommodate the tapered formation of the wedge 22, so that when the wedge 22 is in the position shown in Fig. 4, the said elements will form 105 a substantially cylindrical core. The middle or wedge element 22 is held in operative position by means of the pin 25 at the top of the pouring cup.

It will also be noted that in the structure 110 shown in Fig. 4, the block or core bit 13' is counter-sunk to provide a seat for the outer

elements 21 and 23 of the core, and to form a limit to their expanding or separating movement. This counter-sunk supporting block however in no way interferes with their free contracting movement, or movement toward each other. This block 13' is also provided with the central opening 26 to permit of the downward movement of the wedge element 22, while the other elements 21 and 10 23 are still held in place by said block.

When the mold has been filled with molten metal as described in connection with Figs. 1, 2 and 3, and the billet has become sufficiently set, the pin 25 is withdrawn and 15 the wedge 22 is depressed so as to permit a collapse or moving toward each other of the elements 21 and 23. This serves to allow the contraction of the billet, due to its cooling, without danger of splitting the same.

20 When the billet has sufficiently cooled and contracted the wedge 22 may be moved farther downwardly, or entirely removed from the elements 21 and 23, whereupon the elements 21 and 23 may be ejected or withdrawn 25 from the billet.

In other respects the operation is substantially the same as that described with respect to Figs. 1, 2 and 3.

What I claim is:—

30 1. The method of casting a hollow billet for use in tube drawing which consists in pouring the molten metal into a mold about a resilient metallic core supported vertically on one of its ends and restrained as to its

two ends so that it cannot expand beyond a 35 predetermined maximum but will freely yield to the pressure of the surrounding casting as to its periphery to an extent corresponding to the contraction of the billet upon cooling, and, after the metal of the 40 billet has sufficiently set, removing said billet from the mold with the core therein.

2. In a device of the character described, the combination of an approximately cylindrical mold, a vertically arranged resilient 45 metallic core placed centrally therein, means for supporting the core at its lower end and means for restraining said core as to its two extremities so that it cannot expand beyond a predetermined maximum but will freely 50 yield to the pressure of the surrounding casting to an extent corresponding to the contraction of the billet upon cooling, the parts arranged and proportioned so that the billet with the core inclosed therein may be removed from the mold after the metal of the 55 billet has sufficiently set.

3. The combination of a cylindrical vertically arranged metallic mold, a pouring funnel removably positioned on the top of said 60 mold, a block removably secured within the mold near the bottom thereof, a core, adapted to contract with the contracting metal of the casting, secured within the mold and means including lugs projecting radially 65 from the funnel for limiting the expanding movement of said core.

ROSS EDWARD BRADLEY.